

## UNITED STATES PATENT OFFICE

2,107,605

METHOD OF PRODUCING COLORED PHOTO-  
GRAPHIC MATERIALS

Béla Gáspár, Brussels, Belgium

No Drawing. Application August 9, 1934, Serial  
No. 739,136. In Germany August 10, 1933

6 Claims.

(Cl. 95—7)

It is known to produce photographic materials, which contain an insoluble deposit of a dyestuff with a metal. The production of photographic layers of this nature has not been practicable heretofore, as it has been necessary to introduce the dyestuff into the layer in some complicated manner, or else it has been necessary to produce the dyestuff deposit in the emulsion colloid by way of double conversion, it then being necessary to remove from the layer the products of this double conversion.

This invention relates to a simple and economical method of producing colored photographic materials, in which the substances necessary for the conversion may be introduced into the photographic emulsion without any detrimental effect.

This is accomplished according to the invention by the use of salts of organic acids of that kind in which the anion is unable to act adversely in the photographic layer. Primarily there will be employed salts of metals or organic bases, the cations of which are indifferent in respect to the emulsion, and which result in deposits which are not diffusing, with lake-forming dyestuffs, for example I may use alkaline earth salts, magnesium salts, or certain nitrogenous bases as set forth in my co-pending application now Patent No. 2,046,067, June 30th, 1936.

An additional advantage consists in the fact that I may use the salts of weak acids such as are admirably suitable for puffing of the layer and act favorably on the sensitiveness of the light sensitive layers. Suitable anions for the salts are weak organic acids, such as acetic acid, propionic acid, butyric acid, caproic acid, acrylic acid, malic acid, adipic acid, naphthaline sulfonic acid, maleic acid, aminic acid.

For example, there is admixed with 1 litre of photographic silver bromide emulsion 5 grammes of Chrysophenine G (No. 304 Schultz Farbstofftabelle 5th edition 1920, published by Weidmann Buchhundlung). To this there are added 2 grammes of barium butyrate. On to a layer of this kind there may be poured a second layer, which contains, for example, a red lake-forming dyestuff, such as Antosine BN (Fierz-David: Künstliche organische Farbstoffe, published by Springer, Berlin 1926). For fixing the dyestuff in this case barium butyrate is likewise employed.

The production of a blue filter occurs for example as follows: To a 6% gelatine solution there are added 1% each of Diamine Pure Blue FF (No. 424 Schultz above) and adipic guanidine.

The invention is adaptable therefor both for the coloring of photographic layers and the production of filter layers. The method of the invention may also be employed in conjunction with

separate layers which are situated above or below the light-sensitive layers.

It is accordingly also possible to pour filter layers free of emulsion serving for the screening of photographic emulsion or as a base for photographic layers.

What I claim as new and desire to secure by Letters Patent is:

1. A method of uniformly coloring colloids used in the production of a photographic material including a light sensitive silver halide which comprises causing within the colloid a double decomposition by incorporating a lake forming dyestuff and a salt, which salt contains a lake forming cation and an anion of a colorless weak organic acid, indifferent to the light sensitive silver halide, a dyestuff lake being formed by the reaction and a salt of the weak organic acid resulting as a by-product.

2. A method of uniformly coloring light sensitive silver halide emulsions for photographic purposes which comprises causing within the emulsion a double decomposition by incorporating a lake forming dyestuff and a salt, which salt contains a lake forming cation and an anion of a colorless weak organic acid, indifferent to the light sensitive emulsion, a dyestuff lake being formed by the reaction and a salt of the weak organic acid resulting as a by-product.

3. A method of uniformly coloring colloids to form a colored layer adjacent to a light sensitive silver halide layer in a photographic material which comprises causing within the colloid a double decomposition by incorporating a lake forming dyestuff and a salt, which salt contains a lake forming cation and an anion of a colorless weak organic acid indifferent to the light sensitive layer, a dyestuff lake being formed by the reaction and a salt of the weak organic acid resulting as a by-product.

4. A method of uniformly coloring light sensitive silver halide emulsions for photographic purposes which comprises causing within the emulsion a double decomposition by incorporating a dyestuff, Chrysophenine G, and barium butyrate to form a dyestuff lake.

5. A method of uniformly coloring light sensitive silver halide emulsions for photographic purposes which comprises causing within the emulsion a double decomposition by incorporating a dyestuff, Antosine BN, and barium butyrate to form a dyestuff lake.

6. A method of uniformly coloring light sensitive silver halide emulsions for photographic purposes which comprises causing within the emulsion a double decomposition by incorporating a dyestuff, Diamine Pure Blue FF, and adipic guanidine, to form a dyestuff lake.

BÉLA GÁSPÁR.